

## UNITED STATES PATENT OFFICE

CAMILLE CONTAL, OF ST. CLOUD, FRANCE

## UNOXIDIZABLE ALLOY

No Drawing. Application filed July 17, 1929, Serial No. 379,070, and in France June 21, 1929.

The present invention has for its object an unoxidizable alloy designed particularly for the manufacture of valves and other adjusting and packing members subjected to the action of steam, particularly superheated steam.

This alloy is substantially composed as follows:

|           | Per cent |
|-----------|----------|
| Nickel    | 40 to 50 |
| 10 Copper | 30 to 40 |
| Manganese | 10 to 20 |
| Antimony  | 5 to 15  |
| Tin       | 1 to 10  |

15 By way of example, the following exact proportions give an alloy having all the desirable qualities for the manufacture of the above mentioned articles:

|           |    |
|-----------|----|
| 20 Nickel | 40 |
| Copper    | 31 |
| Manganese | 18 |
| Antimony  | 9  |
| Tin       | 2  |

|          |     |
|----------|-----|
| 25 Total | 100 |
|----------|-----|

For preparing this alloy, use is preferably made of a 30% copper-manganese alloy which is first melted; nickel is then added, 30 and subsequently manganese, antimony and tin. In order to avoid oxidation during melting, a deoxidizing agent for bronze, such as borax, can be added.

The alloy thus obtained has the following 35 properties:

Density: 8.28.

Melting point: about 1000° C.

Texture: Micrographs show that the crystallization is homogeneous.

40 Colour: white.

Hardness: The scleroscopic hardness is of 45 and the hardness as determined by Brinell's method is 210, that is to say a hardness near that of hard steel. If the metal is heated to a temperature of 800° C. and water-hardened it undergoes a material diminution of hardness; the scleroscopic hardness then passes from 55 to 40. Utilization of this phenomenon can facilitate machining.

Resistance to chemical agents: Tests have been effected on a sample having an area of 8 square centimeters; an immersion for 8 hours in boiling potash at 22° Bé. has caused no loss of weight; an immersion for 48 hours in ammonia at 16° Bé. and an exposure during 4 hours to a vapour saturated with ammonia has caused only a loss of weight of 0.005 gr. Boiling nitric and sulphuric acids attack the alloy only with great difficulty. 55

Resistance to the action of steam: It is known that up to now valves, gate valves, etc., as well as the valve seats, exposed to the action of steam, particularly if it is superheated, are corroded after a few days and no longer ensure the necessary fluid-tightness. 60 This corrosive action is both of a chemical and mechanical nature; on the one hand, steam exerts a highly oxidizing action, and it acts, moreover, through the alkaline particles which it frequently contains.

65 However, obturating and adjusting members manufactured from the alloy in accordance with the invention, perfectly resist the passage of superheated steam owing to the great hardness of this alloy and its resistance to the attack of oxidizing and alkaline agents. They have also the advantage of not becoming distorted, as they are not influenced by an increase of temperature to 350° C. 80

This alloy is designed particularly for casting in molds; it may also be easily worked on the lathe and other machine-tools.

An addition of lead, not exceeding 1%, inserted towards the end of the preparation, 85 has the effect of softening the alloy.

It is to be understood that the proportions of the various elements of the alloy can be varied within the limits indicated above and their choice can be easily predetermined in 90 each case so that the required qualities of hardness and unalterability be obtained.

## Claims:

1. Alloy comprising nickel (40 to 50%), copper (30 to 40%), manganese (10 to 20%), antimony (5 to 15%), and tin (1 to 10%). 95
2. Alloy comprising nickel (40 parts), copper (31 parts), manganese (18 parts), antimony (9 parts), tin (2 parts). 100

3. Alloy comprising nickel (40 to 50%), copper (30 to 40%), manganese (10 to 20%), antimony (5 to 15%), tin (1 to 10%), and lead (less than 1%).

5 In testimony whereof I have hereunto affixed my signature.

**CAMILLE CONTAL.**

**10**

**15**

**20**

**25**

**30**

**35**

**40**

**45**

**50**

**55**

**60**

**65**